

2,940,881

**METHOD FOR MAKING CUBE-ON-FACE MAGNETIC STEEL**

John H. Hollomon, Schenectady, N.Y., assignor to General Electric Company, a corporation of New York

No Drawing. Filed Sept. 20, 1956, Ser. No. 610,904

1 Claim. (Cl. 148—111)

This invention relates to magnetically "soft," polycrystalline, body-centered cubic alloys and more particularly to the fabrication of such polycrystalline sheet materials composed of iron, iron and silicon, iron and aluminum, and iron and molybdenum having "cube texture" grain orientation.

As pointed out and particularly disclosed in copending application for United States Letters Patent Serial No. 610,909 of Hibbard and Walter, filed concurrently with this application and assigned to the same assignee, certain alloys of iron have been found to have very desirable magnetic and electrical properties. These materials have been widely used in the form of laminated sheet metal cores and the like for saturable core devices, motors, generators, and other electromagnetic apparatus. The alloys which have the most desirable and useful electrical and magnetic properties have been composed of up to about 5% silicon, balance substantially all iron, up to about 8% aluminum, balance substantially all iron, and up to about 5% molybdenum, balance substantially all iron.

Additionally, it has been found that for certain purposes a strong preferred grain orientation is desirable in sheet and strip material formed by rolling or forging, particularly in the case of silicon steel sheet or strip. This preferred grain orientation has been previously produced in silicon steel, for example, by hot and cold rolling silicon steel ingots into sheets or strips combined with appropriate heat treatment, as is well known in the art. The finished product is, of course, a polycrystalline material which has the body-centered cubic lattice form, and in which a majority of the grains have substantially the same orientation with respect to the plane of the sheet or strip and the direction of rolling. This orientation may be described as one in which the unit cube lattices of the oriented grains have a plane containing diagonally opposite cube edges substantially parallel to the plane of the sheet and a pair of opposite cube faces substantially perpendicular to the rolling direction and to the plane of the sheet. This orientation is conventionally defined and described by metallurgists and crystallographers as the (110) [001] orientation in terms of the Miller Crystallographic Index System, a complete discussion of which may be found, for example, in "Structure of Metals," C. S. Barrett, 2nd Edition, 1952, the Macmillan Company, pages 1 to 25.

As is well known in the art and more particularly set forth in application Serial No. 610,909, previously referenced, this preferred orientation improves the useful magnetic properties of these materials in the plane of the sheet and in the rolling direction, but these magnetic properties in the plane of the sheet and transverse to the rolling direction are comparatively poor.

As disclosed in the previously referenced co-pending application, it has been found that by appropriately rolling and heat treating silicon-iron, molybdenum-iron and aluminum-iron grain oriented castings, a different preferred orientation may be produced in polycrystalline

sheet or strip materials of these compositions. This orientation may be described as one in which a majority of the grains have their body-centered cubic lattices oriented so that four (4) of the cube faces are substantially parallel to the rolling direction, two of these faces being also substantially parallel with the plane of the sheet and the other two being substantially perpendicular to the plane of the sheet, and the remaining two cube faces substantially perpendicular to both the rolling direction and the plane of the sheet. This orientation may

5 be conveniently termed "cube texture" or defined in terms of Miller Indices, (100) [001]. These sheet and strip materials having this orientation have been found to have magnetic properties which are equivalent to those of previously known (110) [001] materials of the same composition in the rolling direction and in the plane of the sheet, and much more desirable magnetic properties in the plane of the sheet transverse to the rolling direction than the previously known materials.

10 As disclosed in the previously reference application, this preferred orientation, i.e., "cube texture," may be produced by particularly preparing cast ingots having an entirely or substantially entirely columnar as-cast grain structure. These castings are produced so that substantially all the metal therein is comprised of elongated columnar grains, the longitudinal axis of each of which is substantially parallel to each other longitudinal grain axis and all of which axes are substantially parallel to a single direction in the ingot. It was found that by ap-

25 propriately hot, warm and cold rolling as-cast slabs of up to about 1 inch in thickness or slabs of that thickness cut from larger ingots, with particular reference to the direction of the longitudinal axes of the columnar grains to the rolling directions and rolling planes that the cold rolled structure of the sheet material so produced could

30 be caused to recrystallize upon appropriate annealing to produce sheet or strip material having the desired cube texture. More specifically, this reduction procedure involved heating such slabs to a temperature range of from

35 about 700° C. to about 1100° C., reducing the thickness of the so-heated slabs about 90 to 97% in a plurality of rolling passes without reheating, annealing, cold reducing the annealing material at least 40% in thickness by cold rolling and annealing to effect recrystallization

40 of the cold rolled grain structure to produce the cube textured sheet or strip material. This casting, rolling and heat treatment procedure was found to be effective to produce cube texture in polycrystalline body-centered cubic sheet or strip materials composed of at least 92% iron and more specifically alloys containing up to about

45 5% silicon, up to about 5% molybdenum and up to about 8% aluminum, all useful soft magnetic materials.

Obviously, a rolling process which depends upon starting with as-cast slabs or slab ingots about 1 inch thick would pose many problems in adaptation to conventional steel mill production procedures. It would be desirable to be able to process much thicker ingots or as-cast sections by rolling without having to first prepare such slabs therefrom.

50 Accordingly, it is a principal object of my invention to provide a process whereby columnar grain ingots or cast intermediates or blanks composed of at least 92% iron and containing up to about 5% silicon or 5% molybdenum or 8% aluminum, and having thicknesses substantially greater than 1 inch may be worked to thinner intermediate thicknesses having a recrystallized cube texture grain structure and subsequently worked to form sheet or strip material of conventional thicknesses and annealed to

55 produce a recrystallized cube texture in the finished product.

An additional object of my invention is the provision

of a rolling and heat treating process whereby silicon-iron, molybdenum-iron and aluminum-iron cube texture sheet or strip material may be produced from ingots composed of columnar as-cast grains without regard to the initial thickness of the starting ingot and without having to perform a slabbing operation upon such ingots.

Other and specifically different objects of my invention will become apparent from the following detailed disclosure.

Briefly stated, in accordance with one embodiment of my invention, I have discovered that the cubic texture in body-centered alloys of iron comprising silicon-iron, molybdenum-iron, and aluminum-iron which may be produced in wrought recrystallized sheet or strip-like bodies of these materials, unexpectedly may be retained through successive working and recrystallization treatments so that there is no limitation save practical or economical considerations on the initial size of the ingot which may be so processed.

Previous investigators have found that polycrystalline iron and body-centered cubic iron alloys, such as, for example, commercial silicon-iron "electrical grade" alloys containing 2 to 5% silicon, less than about 0.005% carbon, balance substantially all iron, including minor amounts of impurities customarily present in such materials, tend to invariably assume certain well known "preferred orientations" or "texture" when subjected to substantial amounts of cold plastic deformation by unidirectional rolling. The cold rolled texture of these materials is chiefly one in which [110] directions of substantially all the grains lie along the direction of rolling, with a deviation of a few degrees, and (001) planes lie in the plane of the rolled sheet, with a deviation from this position chiefly about the rolling direction as an axis. These stable, cold rolled crystal orientations have been identified as (100) [011], (115) [110], (113) [110], (112) [110], (111) [110], (111) [112]. The higher the amount of unidirectional cold reduction given such materials, the greater is the tendency of the grains to assume a (100) [011] orientation in the rolled sheet. This may best be described as an orientation in which a pair of opposite unit cube faces of the body-centered cubic lattices of a majority of the grains in the sheet are substantially parallel to the rolling direction and to the plane of the sheet and a plane containing diagonally opposite cube edges of such unit cubes is substantially perpendicular to the plane of the sheet and substantially parallel to the rolling direction. Upon recrystallization by annealing such cold rolled sheets, the preferred orientation or texture of the annealed sheet will change to an orientation which is different from the cold rolled texture. The annealed preferred orientation of such materials has previously been found to consist of a majority of the grains having a (110) [001] orientation, which has been previously described. It would, therefore, reasonably be expected that when polycrystalline bodies of iron and the body-centered alloys of iron were severely cold rolled in one direction into sheet material the grains comprising such bodies would assume the (100) [011] stable texture or one of the previously mentioned variations thereof, and when recrystallized by annealing, that the annealed texture would be predominantly the (110) [001] orientation usually obtained. I have discovered, however, that contrary to that which would be expected, the plastically deformed structure resulting from unidirectionally cold rolling cube texture polycrystalline iron base alloys of this type recrystallizes into cube texture instead of a predominantly (110) [001] orientation.

Further, I have discovered that once a strong cube texture is obtained in such polycrystalline materials, it may be cold rolled and annealed according to my invention several times in succession, and will still retain the cube texture upon recrystallization after each successive recrystallization anneal.

More specifically, according to my invention, heavy

sectioned grain oriented castings of these materials may be reduced by hot, warm and cold rolling and appropriate heat treatment to produce an intermediate plate-like body having a recrystallized cube texture or (100) [001] orientation, said intermediate body being then further reduced by cold rolling and recrystallization heat treatment to produce either a final sheet or strip product having cube texture, or a yet further intermediate having cube texture which may be cold rolled and recrystallized once or several times more to produce finished sheet or strip material, thereby making it possible to produce such finished material from grain oriented ingots of large size by rolling and heat treating. As illustrative of my invention, a grain oriented casting composed of about 3% by weight silicon, balance substantially all iron was prepared by pouring the molten alloy into a tubular mold of fused alumina, the sidewalls of which were heated to a temperature of about 1400° C. just prior to pouring. The bottom of the mold consisted of a substantially planar water-cooled copper body whose temperature was maintained at about 20° C. whereby substantially all the superheat and latent heat of the molten metal was extracted through said cooled copper bottom during solidification to provide an ingot having an as-cast grain structure substantially consisting of a plurality of elongated columnar grains extending upwardly from the copper bottom, substantially as shown and disclosed in the previously referenced co-pending application.

After cooling, the ingot was cut into a plurality of slabs, each slab having a pair of parallel faces, said faces extending in a direction parallel to the mean direction of the longitudinal axes of the columnar grains, i.e., substantially parallel to the direction of flow of the majority of the heat extracted during solidification of the casting or, in other words, substantially perpendicular to the copper bottom of the mold.

These slabs were reduced by a plurality of rolling passes during which passes the longitudinal axes of the columnar grains were maintained in a direction substantially parallel to the rolling plane and to the rolling direction. After about 70% reduction in thickness of these slabs had been accomplished by cold rolling, certain of these cold rolled bodies were annealed at various times and temperatures and magnetic torque tests were performed on specimens cut therefrom. The results of these torque tests are reproduced in the following table.

Table I

| Anneal Temp., ° C. | Time (Hours) | Maximum Torque, H=1,000 (Ergs per cc.) | Peak Ratio |
|--------------------|--------------|----------------------------------------|------------|
| 800                | 1/2          | 89,300                                 | 0.82       |
| 1,000              | 1/2          | 102,300                                | 0.79       |
| 1,200              | 1/2          | 97,800                                 | 0.90       |
| 800                | 8            | 104,000                                | 0.83       |
| 1,000              | 8            | 94,000                                 | 0.94       |
| 1,200              | 8            | 92,400                                 | 0.70       |
| 800                | 16           | 69,400                                 | 0.76       |
| 1,000              | 16           | 104,700                                | 0.76       |

From the foregoing, as will be appreciated by those skilled in the art, it may be seen that this material had a high degree of cube texture and was produced according to the procedure disclosed in the previously referenced co-pending application.

The remainder of the material having 70% cold reduction was annealed for 8 hours at 1000° C. and certain of these annealed bodies were then subjected to a further 50% reduction in thickness in cold rolling and the remainder of these bodies were then subjected to a further 70% reduction in thickness by cold rolling. These cold rolled bodies were annealed and magnetic torque tests were performed upon specimens cut therefrom.

5  
Table II

| Percent Reduction in Thickness | Anneal Temp., °C. | Time (Hours) | Maximum Torque, H=1,000 (Ergs per cc.) | Peak Ratio |
|--------------------------------|-------------------|--------------|----------------------------------------|------------|
| 50.....                        | 1,000             | 1/2          | 91,400                                 | 0.72       |
|                                | 1,200             | 1/2          | 79,300                                 | 0.68       |
|                                | 800               | 8            | 81,000                                 | 0.81       |
|                                | 1,000             | 8            | 83,600                                 | 0.68       |
|                                | 1,200             | 8            | 91,300                                 | 0.81       |
|                                | 800               | 16           | 54,200                                 | 0.79       |
|                                | 1,000             | 16           | 91,000                                 | 0.70       |
|                                | 1,200             | 1/2          | 101,600                                | 0.87       |
| 70.....                        | 1,200             | 3/2          | 96,800                                 | 0.81       |
|                                | 800               | 8            | 97,000                                 | 0.79       |
|                                | 1,000             | 8            | 81,000                                 | 0.90       |
|                                | 1,200             | 8            | 97,000                                 | 0.80       |
|                                | 800               | 16           | 95,000                                 | 0.86       |
|                                | 1,000             | 16           | 83,000                                 | 0.95       |

From the foregoing test results, it is apparent that the cube texture orientation of these materials may be retained through cold working or recrystallization heat treatments and contrary to that which might reasonably be expected, does not change upon recrystallization to a (110) [001] orientation in any substantial degree.

From this it is apparent that ingots having an as-cast grain orientation consisting of columnar grains as previously disclosed may be reduced from quite heavy as-cast sections to sheet or strip-like material having a recrystallized cube texture without any substantial restriction as to the initial thickness of the ingot. From this, it may be seen that large ingots may be so-cast, rolled and heat treated to form cube texture or strip without having to first reduce said ingots into relatively thin slabs prior to rolling.

For a specific example, assume it is desired to prepare nominal 0.012 inch thick cube texture sheet material of 3% silicon-iron from, for example, a 24" x 24" square, cross section ingot of any appropriate length having substantially all of its as-cast grains in the form of elongated columnar grains whose longitudinal axes extend substantially lengthwise of said ingot.

According to my invention this may be accomplished, for example, in the following manner. The ingot is heated to a temperature of about 1100° C. and rolled without reheating in a plurality of passes to effect about a 90% reduction in thickness to an intermediate slab of about 1.4" thick. During this and subsequent rolling operations the ingot is preferably rolled with its length parallel to the rolling plane and the rolling direction.

This intermediate slab is annealed by heating to about 1000° C. and holding at that temperature for about four hours. The 1.4" thick slab is then cold reduced about 70% by rolling to about 0.42" thick, annealed to a temperature of about 1150° C. and permitted to furnace cool to produce a strong cube texture.

This cube texture material is then further reduced in a plurality of cold rolling steps with interspersed anneals. Preferably the annealing steps are accomplished after a substantial amount of cold reduction, for example, about 50 to 70% has been accomplished. For purposes of this specific example, the 0.42" thick sheet material having cube texture is then cold reduced about 70% to about 0.126" thickness, annealed, for example, for about 8 hours at about 1000° C., cold reduced about 70% to about 0.38" thickness, annealed for about 8 hours at about 1000° C., cold reduced about 70% to about 0.012" thick sheet material and annealed for about 8 hours at about 1000° C. to effect recrystallization of the cold worked crystal structure to cube texture.

It will be appreciated that the foregoing specific illustration involving an ingot having a 24" x 24" square

## 6

cross-section is exemplary only and that other specific sizes and cross-sectional configurations may be equally well employed with appropriate adjustments in the schedule of rolling reductions. Furthermore, the recrystallization of the cold worked structure of these materials may be effected over annealing temperature range of from about 800° C. to over 1200° C. for intervals of time ranging from a few minutes to several, i.e., 8 or more hours, depending primarily upon the particular temperature employed.

It will be appreciated that the specific amounts of rolling reduction and annealing times and temperatures may be varied. For example, it would appear desirable that the amount of cold reduction of thickness before annealing be at least 40% in every case and for commercial considerations may be as large as is convenient. Further, the annealing times and temperatures required after each cold reduction would appear to be quite flexible, ranging from about 1/2 hour at about 1200° C. to as much as 8 hours or more at about 800° C., so long as the cold worked structure is recrystallized.

From the foregoing, it will be apparent that I have invented a method for producing cube texture soft magnetic sheet material composed of alloys consisting of at least 92% iron and up to 5% silicon, up to 5% molybdenum and up to 8% aluminum, by directly processing large commercial size ingots.

What I claim as new and desire to secure by Letters Patent of the United States is:

30 A method for producing polycrystalline sheet-like metal having the body-centered cubic crystal lattice form by rolling and heat treating in which a majority of the grains thereof have the cube texture preferred orientation with respect to the rolling direction and rolling plane 35 of said sheet comprising the steps of rolling a grain oriented ingot composed of a binary alloy selected from the group consisting essentially of up to about 5% silicon, balance substantially all iron, up to about 8% aluminum, balance substantially all iron, and up to about 5% 40 molybdenum, balance substantially all iron to effect a reduction in thickness of at least 40% and form an elongated slab-like body, said ingot being characterized in its as-cast state by being substantially entirely composed of a plurality of elongated columnar grains, the longitudinal 45 axes of which are substantially parallel, said longitudinal grain axes being maintained substantially parallel to the rolling direction and the rolling plane during the rolling operations, annealing said slab at a temperature of from about 800° C. to 1200° C. for a period of time sufficient 50 to effect recrystallization of the cold-worked metal, cold rolling said annealed slab to effect at least a 40% reduction in thickness and form an elongated sheet-like body, annealing said sheet-like body at a temperature of from about 800° C. to 1200° C. for an interval of time sufficient 55 to effect recrystallization in which a majority of the grains have a cube texture preferred orientation, cold rolling said annealed cube texture sheet-like body to effect at least a 40% reduction in thickness, and annealing said sheet-like body at a temperature of from 800° 60 C. to 1200° C. for an interval of time sufficient to effect recrystallization of a majority of the grains of said sheet-like body into the cube texture preferred orientation.

## References Cited in the file of this patent

65 UNITED STATES PATENTS  
2,112,084 Frey et al. ----- Mar. 22, 1938  
2,307,391 Cole et al. ----- Jan. 5, 1943  
2,700,006 Dunn ----- Jan. 18, 1955

## FOREIGN PATENTS

70 610,440 Great Britain ----- Oct. 15, 1948